

# UNITED STATES PATENT OFFICE.

JOHN E. CARNAHAN, OF CANTON, OHIO.

## METHOD OF BLUING STEEL OR IRON SHEETS.

1,141,770.

Specification of Letters Patent.

Patented June 1, 1915.

No Drawing.

Application filed January 2, 1914. Serial No. 809,834.

To all whom it may concern:

Be it known that I, JOHN E. CARNAHAN, a citizen of the United States, residing at Canton, in the county of Stark and State 5 of Ohio, have invented a certain new and useful Method of Bluing Steel or Iron Sheets, of which the following is a specification.

The invention relates to the oxidation of 10 steel or iron sheets for the purpose of giving them a deep or dark blue finish. Ordinary oxidation by steam, air or other oxidizing agent gives them a comparatively light blue finish, which for many purposes is not 15 as desirable or acceptable for commercial purposes as a darker blue finish.

The object of the present invention is attained by oxidizing the surface of the sheets in an annealing box as by the usual steam 20 process, and at the same time subjecting the sheets to the action of sulfur vapor or fumes, which results in giving them a deeper and darker blue than can be produced by the steam or other oxidizing agent alone.

The improved process may be performed 25 by heating the sheets in an annealing box to an annealing heat, and then cooling the sheets while inclosed in the box, to a dark red color, at which time steam or other oxidizing agent is introduced into the box in the usual manner for oxidizing the sheets, and at the same time a small quantity of 30 sulfur is introduced into the annealing box, as by placing it in a small pan and inserting the same under the rim of the annealing box, by raising the box slightly from its bed plate. The sulfur thus introduced into the annealing box may be in powdered, granular, or other convenient form, and may 35 be from several ounces to a pound in weight, according to the size of the box, the surface area of the sheets therein, and the particular depth or darkness of the blue to be produced on the sheets.

Upon the introduction of the sulfur into 45 the box, the heat therein very promptly converts the sulfur into a vapor, and the fumes rising therefrom permeate the pack of sheets and produce in the surface thereof the desired deep or dark blue color. 50

It will be understood that the sulfur can be introduced into the box and will be properly vaporized, at any time while the heat therein is from 1500° F. down to about 700° F., within which range the best results have 55 been obtained; and it will be furthermore understood, that it is not essential to introduce at one time, all the sulfur which may be ultimately required, but the same is preferably introduced at intervals during the 60 cooling of the sheets, and is effective as long as the heat therein properly vaporizes the sulfur.

By the improved method herein described, it has been found that the introduction of 65 sulfur into the annealing box during the period the sheets are being oxidized by the presence of steam or other oxidizing agent therein, the desired deep or dark blue color will be produced in the surface of the sheets 70 without the presence or use of any other element or agent therewith, and without interfering with or impairing the effectiveness of the sulfur fumes for the purpose intended by such other element or agent. 75

I claim:

The method of bluing heated steel or iron sheets which consists in oxidizing the sheets by steam or other oxidizing agent, and at the same time subjecting the sheets 80 to the action of sulfur fumes at a temperature exceeding 700° F.

JOHN E. CARNAHAN.

Witnesses:

EARL C. CARLSON,  
LOUISE M. CORBY.